

## UNITED STATES PATENT OFFICE

2,460,065

## COBALT SULFATE RELATIVE HUMIDITY INDICATORS

Paul Bell Davis, Baltimore, Md., assignor to The Davison Chemical Corporation, Baltimore, Md.

No Drawing. Application February 7, 1945,  
Serial No. 576,716

8 Claims. (Cl. 252—408)

1

This invention relates to indicators and more particularly has reference to compositions for indicating the presence and quantity of moisture in a gaseous atmosphere.

Many chemical compounds and especially a number of salts exist in the anhydrous and hydrated states. A number of these compounds are of one color in the anhydrous state and a different color in the hydrated state and thereby are suitable for use as indicators for detecting the presence of moisture. The above-mentioned compounds, per se, are not suitable for use as quantitative indicators as is contemplated by the present invention but when supported on an adsorbent carrier, as herein described, are highly useful.

In the manufacture of certain products control of the humidity of the air or other gaseous atmosphere is important. It sometimes happens that even a fraction of a percent of relative humidity in an atmosphere may be detrimental to the operation of a process or the product resulting therefrom.

An object of this invention is to indicate the presence of moisture in a gaseous atmosphere at predetermined relative humidities or ranges of relative humidities.

Another object of this invention is to provide a moisture indicator capable of response to the moisture in gaseous atmospheres at predetermined relative humidities.

A further object of this invention is to provide a moisture indicator comprising an adsorbent material having a color changing moisture indicating compound carried thereby.

Still another object of this invention is to provide a moisture indicator comprising an adsorbent material having a color changing moisture indicating compound carried thereby in which the adsorbent characteristics of the carrier, its moisture content, the color-moisture content characteristics of the indicating compound and the concentration thereof are correlated to respond to a predetermined relative humidity of a gaseous atmosphere in contact therewith.

Yet another object of this invention is to provide a moisture indicator comprising a compound which is color responsive to changes in moisture content, carried by silica gel.

It is also an object of this invention to provide a method of making a moisture indicator by depositing a color changing moisture indicating compound in the pores of a porous adsorbent and correlating the character of the adsorbent, its moisture content, and the character and quan-

2

5 tity of the color changing compound to obtain a color response to a predetermined relative humidity of a gaseous atmosphere in contact with the indicator.

With these and other objects in view the present invention resides in the association of a compound, having one color in the anhydrous state and a different color in the hydrated state, with an adsorbent such as silica gel and correlating the character of the adsorbent, its moisture content and the character and content of the color changing compound. Thus by employing an adsorbent having determined adsorbent characteristics and a determined moisture content as a carrier for a quantity of a predetermined compound exhibiting predetermined color changes with relation to the quantity of water associated therewith, and by varying the quantity of the compound and the temperature to which the carrier and compound are heated, an indicator can be obtained which will respond, by a change in color, to a predetermined relative humidity or range of relative humidities of a gaseous atmosphere to which the indicator is exposed.

25 A number of compounds such as cobalt sulphate, cobalt bromide, cobalt phosphate, cobalt chloride, cobalt iodide, cobalt thiocyanate, copper bromide, copper chloride, cobalt fluoro-silicate, and others, change color with changes in 30 the amount of water associated therewith. For example, cobalt chloride in the anhydrous state is of a blue color but when associated with water the color changes. When cobalt chloride has taken up its full water content, it has a pink color.

35 In accordance with the present invention it has been found that by associating a compound, which has one color in the anhydrous state and a different color when combined with water, with 40 an adsorbent, the so treated adsorbent may be employed for indicating the relative humidity of an atmosphere to which the same is exposed.

45 For instance, by impregnating an adsorbent such as silica gel with a solution of cobalt chloride, and drying and activating the so treated silica gel, a product is obtained having a blue color. When the blue colored silica gel is exposed to a humid atmosphere, moisture from the atmosphere is adsorbed by the silica gel and as the water content of the gel is increased the color of the gel gradually changes to pink. The change in color is due to water combining with the anhydrous cobalt chloride in the pores of the gel. It has been discovered according to the present 50 invention that by using a silica gel having cer-

tain adsorptive characteristics, by incorporating a certain amount of cobalt chloride in the gel and by heating the treated gel to a certain temperature, the thus treated gel will change color when exposed to an atmosphere having a relative humidity of a certain minimum value or range of values. It has also been discovered that by changing one or more of the factors, characteristics or conditions, the thus treated gel will respond to a different minimum relative humidity value or range of values. Apart from varying the factors, characteristics, conditions, etc., it has been found that by replacing the cobalt chloride with other chromatic chemicals, color responses to various relative humidities or ranges of relative humidity can be obtained.

Some of the particular chromatic chemicals suitable for use in the present invention will now be discussed.

In the following examples, the values given for the various colors (such as, 5.0 P 4/12) refer to the system of color notation devised by A. H. Munsell and published by Munsell Color Co., Inc., Baltimore, Md., as the Munsell Book of Color, abridged edition, revised 1942.

#### EXAMPLE 1

##### SPECIMEN I-B

Cobalt Sulphate ( $\text{CoSO}_4$ ) is highly useful in practicing the present invention. For instance, standard silica gel made by washing an acid reacting hydrogel with acidic wash water at about 150° F., drying and then activating at about 850° F. and of a size of about 6-16 mesh, has been treated with an aqueous solution of  $\text{CoSO}_4$  of sufficient concentration and in a sufficient amount to incorporate in the gel a deposit of  $\text{CoSO}_4$  of about 2% of the total weight of the gel and  $\text{CoSO}_4$  on a dry basis. After drying at a temperature of about 300° F. and activating at a temperature of about 475° F., the resulting product had a dark purple color or more specifically a Munsell color value of about 5.0 P 4/12.

Upon exposing this product to an atmosphere having a relative humidity between about  $\frac{1}{4}$ - $\frac{1}{2}$ %, the color changed to a dark reddish purple at  $\frac{1}{4}$ % relative humidity, then to a medium red purple at  $\frac{1}{2}$ % relative humidity, or more specifically to a color ranging between 7.5 P 4/8 and 5.0 RP 6/10 M. C. V.

#### EXAMPLE 2

##### SPECIMEN II-B

By varying the temperatures at which the gel containing about 2%  $\text{CoSO}_4$  is dried and activated, a color change or break occurred upon exposing the so treated gel to an atmosphere having a different relative humidity. For instance, upon drying the gel at about 300° F. and activating it at about 850° F. the color will change from 10.0 PB 3/10 Munsell color value to 10.0 P 5/8 M. C. V. when exposed to an atmosphere having a relative humidity of about 3%. Upon exposure to an atmosphere having a relative humidity of about 5% the color will change further to 5.0 RP 6/10 M. C. V.

#### EXAMPLE 3

##### SPECIMEN III-B

If the same gel containing about 2%  $\text{CoSO}_4$  is dried at a temperature of about 300° F. and activated at a temperature of about 600° F., the color will change from 10.0 PB 3/8 Munsell color value to about 7.5 RP 6/10 M. C. V. upon ex-

posure to an atmosphere having a relative humidity of about 5%; and upon further exposure to an atmosphere having a relative humidity up to about 10% the color will change to 10.0 RP 6/10 M. C. V.

#### EXAMPLE 4

##### SPECIMEN II-A

By treating the gel mentioned in Example 1 with a cobalt sulphate solution so that the gel will contain about 2% cobalt sulphate, drying said gel at a temperature of about 350° F. and activating the same at a temperature of about 725° F., an indicator is obtained which is suitable for indicating the moisture content of an atmosphere having a relative humidity ranging between 1% and 3%. For instance, by exposing such a gel having Munsell color value of about 10.0 PB 4/10 to an atmosphere, the relative humidity of which is about 1%, the color will change to about 10.0 P 6/6 M. C. V. and for a relative humidity of about 3% the color will change to about 7.5 RP 7/6 M. C. V.

#### EXAMPLE 5

##### SPECIMEN I-A

By treating the gel mentioned in Example 1 with a cobalt sulphate solution in a quantity calculated to produce a colored gel containing about  $\frac{1}{2}$ % cobalt sulphate, drying the so treated gel at 250° F. and activating the same at about 525° F., an indicator gel will be obtained which has a Munsell color value of about 5.0 P 6/4. Upon exposing this indicator gel to an atmosphere having a relative humidity of about  $\frac{1}{4}$ % the color value will change to about 7.5 RP 7/6 M. C. V. and upon exposing the same to an atmosphere having a relative humidity of about  $\frac{1}{2}$ % the color will change to about 10.0 RP 7/6 M. C. V.

#### EXAMPLE 6

##### SPECIMEN IV-B

A moisture indicator responsive to relative humidities between 5 to 10% was prepared by treating a gel similar to that set forth in Example 1 but which had been washed with water at a temperature of about 175° F., dried and then activated at about 1200° F. and sized to 6-12 mesh, with a quantity of cobalt sulphate solution calculated to impregnate the gel with about 3% cobalt sulphate. Upon drying the so treated gel at a temperature of about 300° F. and activating the same at a temperature of about 1000° F. a product was produced having a Munsell color value of about 10.0 PB 3/10. Upon exposing the so treated gel to an atmosphere having a relative humidity of about 5% the color changed to about 10.0 P 4/8 M. C. V. and upon exposing the gel to an atmosphere having a relative humidity of about 10%, the color further changed to about 5.0 RP 6/10 M. C. V.

#### EXAMPLE 7

##### SPECIMEN III-A

It has been found that copper bromide ( $\text{CuBr}_2$ ) is also suitable for use as an indicator when associated with silica gel. By treating a silica gel such as disclosed in Example 1 with a copper bromide solution in a quantity sufficient to incorporate about 4%  $\text{CuBr}_2$  in the gel, drying the so treated gel at 250° F. and activating the same at about 600° F., a product is obtained having a Munsell color value of about 5.0 GY 2/2. Upon exposing the so treated gel to an atmosphere

having a relative humidity of about 5% the color will change to about 5.0 G 5/8 M. C. V. Upon exposing the gel to an atmosphere having a relative humidity of about 10% the color will change to 10.0 G 5/6 M. C. V.

#### EXAMPLE 8

##### SPECIMEN VIII-A

If a copper bromide impregnated gel corresponding to that of Example 7 and having a  $\text{CuBr}_2$  content of about 4% is dried at about 250° F. and activated at a temperature of about 350° F., a product is obtained having a Munsell color value of about 10.0 YR 2/2. If this product is exposed to an atmosphere having a relative humidity of about 20% the color will change to about 2.5 GY 4/4 M. C. V. If the product is exposed to an atmosphere having a relative humidity of about 30% the color will change to about 2.5 G 6/6 M. C. V.

#### EXAMPLE 9

##### SPECIMEN IV-A

Cobalt bromide ( $\text{CoBr}_2$ ) is a suitable compound for association with a silica gel for the production of an indicator. For instance, by treating a silica gel such as described in Example 1 with a solution of cobalt bromide in a quantity and having a concentration sufficient to impregnate the gel to an extent of about 3/4%  $\text{CoBr}_2$ , drying the product at a temperature of about 275° F. and activating at 400° F., a product is obtained having a Munsell color value of about 5.0 B 3/6. Upon exposing this product to an atmosphere having a relative humidity of about 5%, the color will change to about 7.5 B 7/2 M. C. V. Upon exposing the indicator to an atmosphere having a relative humidity of about 10%, the color will change to 7.5 R 8/4 M. C. V.

#### EXAMPLE 10

##### SPECIMEN VI-A

By impregnating the silica gel of Example 1 with a solution of cobalt bromide of such quantity and concentration as to impregnate the gel to an extent of about 2%  $\text{CoBr}_2$ , and drying the same at a temperature of about 200° F., a product is obtained having a Munsell color value of about 10.0 GY 3/4. Upon exposing this product to an atmosphere having a relative humidity of about 10% the color changed to about 5.0 YR 7/8 M. C. V. Upon exposing the product to an atmosphere, the relative humidity of which is about 20%, the color changed to about 2.5 YR 7/6 M. C. V.

#### EXAMPLE 11

##### SPECIMEN VII-B

By preparing an indicator gel from silica gel corresponding to that used in Example 1 and impregnating the same with a quantity of cobalt bromide to an extent of about 3% and drying the same at a temperature of about 200° F., a product is obtained having a Munsell color value of about 2.5 G 3/4. Upon exposing this product to an atmosphere having a relative humidity of about 10% the color changed to about 10.0 YR 5/8 M. C. V. Upon exposing the product of this example to an atmosphere having a relative humidity of about 20% the color changed to 2.5 YR 5/10 M. C. V.

#### EXAMPLE 12

##### SPECIMEN IX-B

A silica gel such as that described in Example 5 1 was impregnated with cobalt bromide to a content of about 2%  $\text{CoBr}_2$ . Upon drying this product at a temperature of about 250° F., a product was obtained having a Munsell color value of about 7.5 YR 3/2. The color of this compound changed to about 2.5 GY 6/4 M. C. V. upon exposing it to an atmosphere having a relative humidity of about 20%. When the product of this example was exposed to an atmosphere having a relative humidity of about 40% the color changed to about 15 7.5 G 7/6 M. C. V.

#### EXAMPLE 13

##### SPECIMEN V-A

Cobalt phosphate has also been found useful as a chromatic chemical for association with silica gel for the preparation of an indicator in accordance with the present invention. By impregnating a silica gel such as described in Example 1 with cobalt phosphate to an extent 20 25 whereby the product has a  $\text{Co}_3(\text{PO}_4)_2$  content of about 1/2%, drying the product at about 250° F. and activating it at a temperature of about 400° F., an indicator gel was obtained having a Munsell color value of about 7.5 PB 3/10. Upon 30 35 exposing this product to an atmosphere having a relative humidity of about 10% the color changed to about 5.0 R 8/4 M. C. V. When the product was exposed to an atmosphere having a relative humidity of about 20% the color changed to about 2.5 R 8/4 M. C. V.

#### EXAMPLE 14

##### SPECIMEN V-B

Cobalt chloride may be used in various concentrations for association with silica gel for the production of moisture indicators in accordance with the present invention. By incorporating cobalt chloride with a silica gel such as described 40 45 in connection with Example 1 to such an extent that the product has a  $\text{CoCl}_2$  content of about 1/2%, drying the product at a temperature of about 300° F. and activating it at 400° F., an indicator gel was obtained the Munsell color value of which is about 5.0 PB 4/10. When this indicator gel was exposed to an atmosphere having a relative humidity of about 10% the color changed to about 7.5 RP 8/2 M. C. V. This indicator gel had the same color even when exposed to an atmosphere having a relative humidity of about 20%.

#### EXAMPLE 15

##### SPECIMEN VII-A

60 By preparing an indicator gel from silica gel and cobalt chloride, such that it had a  $\text{CoCl}_2$  content of about 2% and drying the same at a temperature of about 200° F., an indicator gel was obtained having a Munsell color value of about 5.0 PB 3/12. When this indicator was exposed to an atmosphere having a relative humidity of about 10%, the color changed to about 7.5 PB 5/10 M. C. V. Upon exposing the indicator to an atmosphere having a relative humidity of about 20% the color changed to about 10.0 RP 6/8 M. C. V.

#### EXAMPLE 16

##### SPECIMEN X-B

75 By treating a silica gel similar to that of

Example 1 but which had been activated at a temperature of about 1100° F. with cobalt chloride in a quantity sufficient to have a 5%  $\text{CoCl}_2$  content, drying the same at a temperature of about 300° F. and activating at a temperature of about 400° F., an indicator gel was obtained having a Munsell color value of about 7.5 PB 2/6. Upon exposing this product to an atmosphere having a relative humidity of about 40%, the color changed to 10.0 P 4/8 M. C. V. The same indicator exposed to an atmosphere having a relative humidity of about 60% exhibited a color of about 7.5 RP 5/8 M. C. V.

EXAMPLE 17

SPECIMEN VI-B

Copper chloride is another chromatic chemical suitable for use in accordance with the present invention. By impregnating silica gel prepared in accordance with that described in Example 1 with copper chloride to an extent whereby the resulting indicator gel has a  $\text{CuCl}_2$  content of about 2%, drying at a temperature of about 300° F. and activating at a temperature of about 600° F., a product was obtained having a Munsell color value of about 7.5 GY 4/6. Upon exposing this indicator gel to an atmosphere having a relative humidity of about 10% the color changed to about 10.0 GY 7/8 M. C. V. and upon exposing the product to an atmosphere having a relative humidity of about 20%, the color changed to about 2.5 G 7/8 M. C. V.

EXAMPLE 18

SPECIMEN VIII-B

Cobalt iodide was incorporated with a silica gel such as that described in Example 1 so as to produce an indicator gel having a  $\text{CoI}_2$  content of about 2%. Upon drying this product at a temperature of about 250° F. and activating it at a temperature of about 400° F., an indicator gel was obtained, the Munsell color value of which was about 7.5 PB 2/4. When this indicator gel was exposed to an atmosphere having a relative humidity of about 20%, the color changed to 7.5 GY 5/2 M. C. V. When the same product was exposed to an atmosphere having a relative humidity of about 30%, the color changed to about 10.0 PB 6/2 M. C. V.

EXAMPLE 19

SPECIMEN X-A

By heating a silica gel having a cobalt iodide content of about 2% to a drying temperature of about 250° F., an indicator gel was obtained having a Munsell color value of about 7.5 GY 2/2. This indicator gel changed its color upon exposure to an atmosphere, having a relative humidity of about 40%, to about 2.5 Y. 6/6 M. C. V. When this same indicator gel was exposed to an atmosphere having a relative humidity of about 60%, the color changed to 2/5 YR 7/4 M. C. V.

EXAMPLE 20

SPECIMEN IX-A

By treating a silica gel such as that described in Example 1 with cobalt thiocyanate to produce an indicator gel having a  $\text{Co}(\text{SCN})_2$  content of about 3/4% and drying the same at a temperature of about 250° F., an indicator gel was obtained having a Munsell color value of about 7.5 PB 3/14. The color of this compound changed to about 10.0 PB 5/8 M. C. V. upon exposure to

an atmosphere having a relative humidity of about 20%. Upon exposing the same compound to an atmosphere having a relative humidity of about 40% the color further changed to about 7.5 RP 6/8 M. C. V.

Many of the indicator gels prepared according to the present invention have high adsorptive characteristics, especially those which are activated after drying and these may be employed for the same purposes as ordinary desiccant silica gel as well as for moisture indicators. Of course, some of the indicator gels, especially those in which drying without activation is employed to correlate the moisture content with the other factors and characteristics, do not have the adsorptive capacity of desiccant silica gel. These indicator gels therefore are used principally for moisture indicating purposes. In some instances such indicator gels may be dispersed through masses of desiccant silica gel having high adsorptive capacities to indicate when the desiccant silica gel has taken up a predetermined quantity of moisture.

In impregnating the silica gel with the solution of chromatic chemical, the gel was first subjected to an atmosphere having a high relative humidity to saturate the gel with moisture to such an extent that upon contacting the same with a liquid the gel would not disintegrate, which happens upon contacting freshly activated gel with a liquid. Also by saturating the gel to approximately 30% total volatile matter, only about 50 ml. of solution is required to wet about 1 kilogram of gel. As before indicated, the concentration of the solution of chromatic chemical is such that by wetting the saturated gel with the above mentioned quantity of solution per kilogram of gel, the desired concentration of chemical in the gel is obtained.

By holding the gel at the drying temperatures indicated in the preceding examples, effective drying is accomplished. Also by holding the gel at the activating temperatures mentioned activation is effected. In each instance, the indicator gel was held at the drying and/or activating temperatures for about three hours.

While the indicators have been described as including carriers of silica gel impregnated with a chromatic chemical, it should be understood that other adsorbent carriers may be used. For instance, a porous adsorbent glass which is described in the Hood et al. Patents Nos. 2,106,744, 2,315,328 and 2,315,329, may be used as set forth in my copending application Serial No. 576,726, (now abandoned), filed of even date herewith.

To demonstrate the utility and practicability of the present invention, a specimen set of indicator gels was made and sealed in small glass ampules. Each specimen consisted of three tubes or ampules, one containing a portion of a certain indicator gel before exposure to an atmosphere, the relative humidity of which was to be determined, the second containing a portion of the same indicator gel after exposure to an atmosphere having a predetermined relative humidity, and the third containing a portion of the same indicator gel after exposure to an atmosphere having a higher relative humidity. Apart from demonstrating the color changes or breaks, these specimens are useful as standards for comparison of the colors of indicator gels exposed to atmospheres having unknown relative humidities.

Two sets of specimens were arranged in frames for convenience in handling and the

frames were designated by Roman numerals and the specimens in each frame were designated by the letters A and B.

The following Table I designates the constitution of the indicator gels of the specimens and Table II designates the colors of the indicator gels before and after exposure to two atmospheres of different relative humidities, the humidities being those at which the colors distinctly change.

In the preceding examples and in Table II, colors are described for the indicator gels when exposed to two atmospheres of different relative humidities. However, these two specific relative humidities are to be taken as the upper and lower limits of a range in which a distinctive color break will occur, the color changing from that for the activated indicator gel to a color within the range of colors, the limits of which are indicated.

Data concerning the various specimens of indicator gels prepared in accordance with the present invention are given in the following tables:

Table I  
INDEX TO SPECIMEN SET OF INDICATING GELS

| Frame No. | Color Break (Relative Humidity) | Indicator Gel No.             | Gel        | Indicator                                       | Per Cent Indicator | Dried at— | Activated at— | ° F. | ° F. |
|-----------|---------------------------------|-------------------------------|------------|-------------------------------------------------|--------------------|-----------|---------------|------|------|
| I.....    | (A. 0%—1/4%<br>B. 1/4%—1/2%)    | 214<br>97-3A-475<br>97-3B-725 | 85956-160  | CoSO <sub>4</sub>                               | 1/2                | 250       | 525           |      |      |
|           | (A. 1/4%—1/2%)                  |                               | 85956-160  | do                                              | 2                  | 300       | 475           |      |      |
| II.....   | (A. 1-3<br>B. 3-5               | 97-2                          | 85956-160  | do                                              | 2                  | 350       | 725           |      |      |
|           | (A. 0-5                         |                               | 85956-160  | CuBr <sub>2</sub>                               | 4                  | 250       | 600           |      |      |
| III.....  | (A. 0-5                         | 110                           | 85956-160  | CoSO <sub>4</sub>                               | 2                  | 300       | 600           |      |      |
|           | (A. 5-10                        |                               | 85956-160  | CoBr <sub>2</sub>                               | 3/4                | 275       | 400           |      |      |
| IV.....   | (B. 5-10                        | 112                           | 129756-120 | CoSO <sub>4</sub>                               | 3                  | 300       | 1000          |      |      |
|           | (A. 0-10                        |                               | 85956-160  | Co <sub>3</sub> (PO <sub>4</sub> ) <sub>2</sub> | 1/2                | 250       | 400           |      |      |
| V.....    | (B. 0-10                        | 194-A                         | 85956-160  | CoCl <sub>2</sub>                               | 1/2                | 300       | 400           |      |      |
|           | (A. 0-10                        |                               | 85956-160  | CoBr <sub>2</sub>                               | 2                  | 200       | -----         |      |      |
| VI.....   | (B. 0-10                        | 169                           | 85956-160  | CuCl <sub>2</sub>                               | 2                  | 300       | 600           |      |      |
|           | (A. 10-20                       |                               | 85956-160  | do                                              | 2                  | 200       | -----         |      |      |
| VII.....  | (B. 10-20                       | 171                           | 85956-160  | CoBr <sub>2</sub>                               | 3.0                | 200       | -----         |      |      |
|           | (A. 10-20                       |                               | 85956-160  | CuBr <sub>2</sub>                               | 4                  | 250       | 350           |      |      |
| VIII..... | (A. 20-30                       | 49                            | 85956-160  | CoI <sub>2</sub>                                | 2                  | 250       | 400           |      |      |
|           | (B. 20-30                       |                               | 85956-160  | CoI <sub>2</sub>                                | 2                  | 250       | 400           |      |      |
| IX.....   | (A. 20-40                       | 211                           | 85956-160  | Co(SCN) <sub>2</sub>                            | 3/4                | 250       | -----         |      |      |
|           | (B. 20-40                       |                               | 85956-160  | CoBr <sub>2</sub>                               | 2                  | 250       | -----         |      |      |
| X.....    | (A. 40-60                       | 165                           | 85956-160  | CoI <sub>2</sub>                                | 2                  | 250       | -----         |      |      |
|           | (B. 40-60                       |                               | 164        | 85956-160                                       | CoCl <sub>2</sub>  | 5         | 300           | 400  |      |
|           |                                 | 141                           | 11956-160  | CoCl <sub>2</sub>                               |                    |           |               |      |      |

Table II  
APPROXIMATE MUNSELL COLOR VALUE (M. C. V.) OF SPECIMEN SET OF INDICATING GELS

| Frame No. | Relative Humidity | M. C. V.     | Relative Humidity | M. C. V.    | Relative Humidity | M. C. V.     |
|-----------|-------------------|--------------|-------------------|-------------|-------------------|--------------|
| I.....    | (A. Activated     | 5.0 P 6/4    | 1/4               | 7.5 RP 7/6  | 1/2               | 10.0 RP 7/6  |
|           | (B. Activated     | 5.0 P 4/12   |                   | 7.5 P 4/8   |                   | 5.0 RP 6/10  |
| II.....   | (A. Activated     | 10.0 PB 4/10 | 1                 | 10.0 P 6/6  | 3                 | 7.5 RP 7/6   |
|           | (B. Activated     | 10.0 PB 3/10 |                   | 10.0 P 5/8  |                   | 5.0 RP 6/10  |
| III.....  | (A. Activated     | 5.0 GY 2/2   | 5                 | 5.0 G 5/8   | 10                | 10.0 G 5/6   |
|           | (B. Activated     | 10.0 PB 3/8  |                   | 7.5 RP 6/10 |                   | 10.0 RP 6/10 |
| IV.....   | (A. Activated     | 5.0 B 3/6    | 5                 | 7.5 B 7/2   | 10                | 7.5 R 8/4    |
|           | (B. Activated     | 10.0 PB 3/10 |                   | 10.0 P 4/8  |                   | 5.0 RP 6/10  |
| V.....    | (A. Activated     | 7.5 PB 3/10  | 10                | 5.0 R 8/4   | 20                | 2.5 R 8/4    |
|           | (B. Activated     | 5.0 PB 4/10  |                   | 7.5 RP 8/2  |                   | 7.5 RP 8/2   |
| VI.....   | (A. Activated     | 10.0 GY 3/4  | 10                | 5.0 YR 7/8  | 20                | 2.5 YR 7/6   |
|           | (B. Activated     | 7.5 GY 4/6   |                   | 10.0 GY 7/8 |                   | 2.5 G 7/8    |
| VII.....  | (A. Activated     | 5.0 PB 3/12  | 10                | 7.5 PB 5/10 | 20                | 10.0 R 6/8   |
|           | (B. Activated     | 2.5 G 3/4    |                   | 10.0 YR 5/8 |                   | 2.5 YR 5/10  |
| VIII..... | (A. Activated     | 10.0 YR 2/2  | 20                | 2.5 GY 4/4  | 30                | 2.5 G 6/6    |
|           | (B. Activated     | 7.5 PB 2/4   |                   | 7.5 GY 5/2  |                   | 10.0 PB 6/2  |
| IX.....   | (A. Activated     | 7.5 PB 3/14  | 20                | 10.0 PB 5/8 | 40                | 7.5 RP 6/8   |
|           | (B. Activated     | 7.5 YR 3/2   |                   | 2.5 GY 6/4  |                   | 7.5 G 7/6    |
| X.....    | (A. Activated     | 7.5 GY 2/2   | 40                | 2.5 Y 6/6   | 60                | 2.5 YR 7/4   |
|           | (B. Activated     | 7.5 PB 2/8   |                   | 10.0 P 4/6  |                   | 7.5 RP 5/8   |

In using the moisture indicator of the present invention, a gel impregnated with a determined quantity of a selected chromatic chemical is dried, or dried and activated, at predetermined temperatures to produce an indicator having its characteristics, etc., correlated to change color upon exposure to a gaseous atmosphere such as

70 to 3% on a dry basis, of cobalt sulphate, said cobalt sulphate having one color in a hydrated state and a different color in a less hydrated state, and heat treating the so impregnated silica at 250-1000° F., said indicator changing color when exposed to an atmosphere having a relative humidity of 0-10%.

2. A quantitative relative humidity indicator as prepared by the method of claim 1.

3. A method of preparing a quantitative relative humidity indicator comprising impregnating activated silica gel without about  $\frac{1}{2}\%$ , on a dry basis, of cobalt sulphate, drying the impregnated silica gel at a temperature of about  $250^{\circ}$  F., and activating the impregnated silica gel at a temperature of about  $525^{\circ}$  F., said indicator changing color when exposed to an atmosphere having a relative humidity of  $0\text{--}\frac{1}{4}\%$ .

4. A quantitative relative humidity indicator consisting essentially of silica gel impregnated with about  $\frac{1}{2}\%$ , on a dry basis, of cobalt sulphate, said indicator changing color when exposed to an atmosphere having a relative humidity ranging from zero to  $\frac{1}{4}\%$  and being prepared by the method of claim 3.

5. A method of preparing a quantitative relative humidity indicator comprising impregnating activated silica gel with about 2%, on a dry basis, of cobalt sulphate, drying the impregnated silica gel at a temperature of about  $300^{\circ}$  F., and activating the impregnated silica gel at a temperature of about  $475^{\circ}$ , said indicator changing color when exposed to an atmosphere having a relative humidity of  $\frac{1}{4}$  to  $\frac{1}{2}\%$ .

6. A quantitative relative humidity indicator consisting essentially of silica gel impregnated with about 2%, on a dry basis, said indicator changing color when exposed to an atmosphere having a relative humidity ranging from  $\frac{1}{4}$  to  $\frac{1}{2}\%$  and being prepared by the method of claim 5.

7. A method of preparing a quantitative relative humidity indicator comprising impregnating

activated silica gel with about 3%, on a dry basis, of cobalt sulphate, drying the impregnated silica gel at a temperature of about  $300^{\circ}$  F., and activating the impregnated silica gel at a temperature of about  $1000^{\circ}$  F., said indicator changing color when exposed to an atmosphere having a relative humidity of 5-10%.

8. A quantitative relative humidity indicator consisting essentially of silica gel impregnated with about 3%, on a dry basis, of cobalt sulphate, said indicator changing color when exposed to an atmosphere having a relative humidity ranging from 5 to 10% and being prepared by the method of claim 7.

15 PAUL BELL DAVIS.

#### REFERENCES CITED

The following references are of record in the file of this patent:

#### UNITED STATES PATENTS

| Number    | Name                  | Date           |
|-----------|-----------------------|----------------|
| 1,947,381 | Connolly et al. ----- | Feb. 13, 1934  |
| 1,976,875 | Connolly et al. ----- | Oct. 16, 1934  |
| 2,210,862 | Tronstad -----        | Aug. 6, 1940   |
| 2,214,354 | Snelling -----        | Sept. 10, 1940 |

#### FOREIGN PATENTS

| Number  | Country             | Date          |
|---------|---------------------|---------------|
| 393,094 | Great Britain ----- | June 1, 1933  |
| 280,934 | Great Britain ----- | Feb. 18, 1929 |

#### OTHER REFERENCES

The Chemical Trade Journal and Chemical Engineer, July 14, 1939, page 31.

**Certificate of Correction**

Patent No. 2,460,065.

January 25, 1949.

**PAUL BELL DAVIS**

It is hereby certified that errors appear in the printed specification of the above numbered patent requiring correction as follows:

Column 7, line 7, example 16, for "Munsell color value of about 7.5 PB 2/6." read *Munsell color value of about 7.5 PB 2/8.*; line 10, same example, for "changed to 10.0 P 4/8" read *changed to 10.0 P 4/6*; and that the said Letters Patent should be read with these corrections therein that the same may conform to the record of the case in the Patent Office.

Signed and sealed this 31st day of May, A. D. 1949.

[SEAL]

**THOMAS F. MURPHY,**  
*Assistant Commissioner of Patents.*